

Oct. 16, 1951

D. B. KIMBALL ET AL

2,571,725

ELIMINATING STAIN IN PHOTOGRAPHIC COLOR MATERIAL

Filed Aug. 15, 1946



DONALD B. KIMBALL  
WENDELL H. McDOWELL  
INVENTORS

BY *Newton M. Perrine*  
*R. Frank Smith*  
ATTORNEYS

## UNITED STATES PATENT OFFICE

2,571,725

## ELIMINATING STAIN IN PHOTOGRAPHIC COLOR MATERIAL

Donald B. Kimball and Wendell H. McDowell,  
Rochester, N. Y., assignors to Eastman Kodak  
Company, Rochester, N. Y., a corporation of  
New Jersey

Application August 15, 1946, Serial No. 690,720

2 Claims. (Cl. 95—8)

1

This invention relates to photography and particularly to a method of eliminating stain in photographic color material.

In the production of colored images in photographic emulsions containing color-forming compounds, the composition of the support material, especially paper, affects the quality and stability of the colored images. For example, photographic paper frequently contains formaldehyde which is used in the production of the paper, and this may cause stain or otherwise adversely affect the photographic emulsion coated on the paper support. Loss in emulsion density may also be caused for this, or other reason.

It is therefore an object of the present invention to provide a method for eliminating stain and emulsion density loss in photographic emulsions containing color-forming compounds. A further object is to provide a method of preventing color falsification or degradation, and to preserve proper color rendition, in a photographic element having emulsions containing color-forming compounds. A still further object is to provide a method for overcoming the adverse effect of formaldehyde on photographic color emulsions. Other objects will appear from the following description of the invention.

These objects are accomplished by incorporating in a layer of the photographic element, such as a baryta layer on paper, an alkali metal sulfite or bisulfite or an aldehyde bisulfite. The sulfite or bisulfite may also be incorporated in the support material itself or in a backing layer or intermediate layer of the photographic element.

The accompanying drawing is a sectional view of a photographic element constructed according to our invention.

According to the preferred form of our invention, photographic paper stock, which may or may not contain an aldehyde having adverse effect on the color-forming emulsion layers coated on the support, is coated with a baryta layer containing an alkali metal sulfite or bisulfite or an aldehyde bisulfite. A subbing layer or layers may then be applied, if desired, followed by one or more silver halide emulsion layers containing color-forming compounds.

The compounds used in the baryta coating may consist of an alkali metal sulfite or bisulfite such as sodium, potassium or ammonium sulfite or bisulfite or an aldehyde bisulfite such as acetaldehyde bisulfite. The aldehyde combined with the bisulfite is not in free form and, therefore, does not adversely affect the color-forming emulsion layer.

2

The sulfites or bisulfites may be incorporated in the paper itself or in a backing layer or an intermediate layer of the photographic element. They may also be applied to elements having supports other than paper, such as cellulose esters or synthetic resin supports.

The color-forming compounds incorporated in the emulsion layer or layers of the photographic element may include any of the known coupler compounds such as those described in Vittum, Peterson and Porter, U. S. Patents Nos. 2,271,238; 2,362,598; and 2,353,205; Weissberger U. S. Patent No. 2,298,443 and Salminen, Weissberger and Glass U. S. Patent No. 2,313,586. In the case of multi-layer coatings the emulsion layers are usually coated with the red sensitive layer containing the cyan coupler nearest the support, the green sensitive layer containing the magenta layer next, and the blue sensitive layer containing the yellow coupler outermost.

Upon storage of a multi-layer photographic paper containing couplers producing yellow, magenta, and cyan dye images, there is a tendency for a loss of yellow emulsion density, and there is also a propensity towards cyan dye stain. The sulfites and bisulfites which we propose to use prevent loss of yellow emulsion density and also prevent the formation of cyan or yellow dye stain.

Our invention will be illustrated by reference to the following example.

To 100 pounds of baryta formula containing 39% solids there were added 112 grams of sodium bisulfite. This combination was coated on photographic paper stock so as to obtain 0.2 gram of bisulfite per square meter of paper when the total weight of coating was 30 grams per square meter. Following this a coating of about 25 grams per square meter of baryta was applied from a formula containing no sodium bisulfite. By applying the baryta in two layers the advantages of the sulfite were achieved and better adhesion of the emulsion layers was obtained. The usual emulsion layers containing couplers were then applied, and it was found that the material had high stability to heat and moisture when compared with similar products containing no bisulfite.

While this coating contained 0.2 gram of sodium bisulfite per square meter of surface, it was found that amounts as low as 0.05 gram per square meter of surface were effective in improving the emulsion stability. Amounts greater than 0.2 gram per square meter of surface can, of course, be used but higher amounts of bisulfite tend to decrease the adhesion of the emulsion layers to the support.

In the accompanying drawing which illustrate the preferred form of our invention in sectional view, 10 is a support of paper or other material which may or may not contain formaldehyde, 11 is a baryta layer containing the alkali metal sulfite or bisulfite or the aldehyde bisulfite, followed by the customary emulsion layers 12, 13 and 14 containing coupler or color-forming compounds. The usual yellow filter layer 15 is coated between the layers 13 and 14. 10

The sulfites may also be incorporated in the support or the baryta layer of a photographic element not containing couplers, in order to prevent loss in emulsion density.

It will be understood that the examples and modifications discussed herein are illustrative only, and that our invention is to be taken as limited only by the scope of the appended claims.

What we claim and desire to secure by Letters Patent of the United States is:

1. A photographic element comprising a paper support having thereon at least one silver halide emulsion layer containing a color former capable of reacting with the development product of a primary aromatic amino developing agent to produce a dye image in said emulsion layer, a paper support containing an aldehyde tending to react to produce color fog and a baryta layer between said paper support and said emulsion layer containing an alkali metal sulfite acting to prevent formation of color fog. 25 30

2. A photographic element comprising a paper support having thereon at least one silver halide emulsion layer containing a color former capable of reacting with the development product of an aromatic amino agent to produce a dye image in said emulsion layer, a paper support containing an aldehyde tending to react to produce color fog and a baryta layer between said paper support and said emulsion layer containing sodium bisulfite acting to prevent formation of color fog. 5 10

DONALD B. KIMBALL.  
WENDELL H. McDOWELL.

#### REFERENCES CITED

15 The following references are of record in the file of this patent:

#### UNITED STATES PATENTS

| Number       | Name          | Date          |
|--------------|---------------|---------------|
| 20 1,763,533 | Miller        | June 10, 1930 |
| 1,954,452    | Mannes et al. | Apr. 10, 1934 |
| 2,304,940    | Mannes et al. | Dec. 15, 1942 |
| 2,309,492    | Albers et al. | Jan. 26, 1943 |
| 2,360,290    | Vittum et al. | Oct. 10, 1944 |

#### FOREIGN PATENTS

| Number    | Country       | Date    |
|-----------|---------------|---------|
| 25 13,835 | Great Britain | of 1907 |

#### OTHER REFERENCES

30 British Journal of Photography, vol. 75, Mar. 23, 1928, pp. 172-173.